

No. 785,167.

PATENTED MAR. 21, 1905.

E. HEDBURG,

## PROCESS OF SEPARATING AND REFINING COMPLEX ORES

APPLICATION FILED JAN 15 1904



*Witnesses:*

Oliver Plumtree

Robert T. Weir

Inventor:  
Eric Hedberg.  
By John W. Hill  
Attorney.

## UNITED STATES PATENT OFFICE.

ERIC HEDBURG, OF JOPLIN, MISSOURI, ASSIGNOR, BY MESNE ASSIGNMENTS, TO AMERICAN REDUCTION COMPANY, OF CHICAGO, ILLINOIS, A CORPORATION OF ARIZONA TERRITORY.

## PROCESS OF SEPARATING AND REFINING COMPLEX ORES.

SPECIFICATION forming part of Letters Patent No. 785,167, dated March 21, 1905.

Application filed January 15, 1904. Serial No. 189,082.

*To all whom it may concern:*

Be it known that I, ERIC HEDBURG, a citizen of the United States, and a resident of Joplin, in the county of Jasper and State of Missouri, have invented a new and useful Process of Separating and Refining Complex Ores, of which the following is a description.

Heretofore various mines and dumps containing complex ores and tailings have been workable only at a loss or, at best, a small profit. By my hereinafter-described process such mines or dumps may be profitably worked. In this process the ores after being roasted are subjected to the action of a hydrocarbon gas, the effect of which is that the copper, nickel, and iron ores become magnetized, while the zinc ores remain non-magnetic, after which the ores are separated by my improved magnetic separators.

The first preliminary step in the process is to crush the ores or concentrates to a degree of fineness sufficient to disengage the various mineral combinations. Next, the ores if not containing a sufficient quantity—for example, substantially ten per cent.—of lime or baryta or baryta sulfate are mixed with a portion of lime to facilitate the elimination of sulfur in the process of roasting (as lime takes up sulfur when heated therewith) and also prevent overheating of the ores; but if the ores already contain a sufficient quantity—for example, more than ten per cent.—of lime or baryta a portion of carbonaceous powder, such as crushed coke or charcoal, is added to the ore to neutralize the excess of lime and eliminate the sulfur of baryta. The ores having been fluxed to a proper consistency are charged into a drier and thence into a roasting-furnace, in which they are subjected to a slightly-oxidizing roast, which transforms the copper and nickel sulfids into a calcic oxid and calcic ferrite, the baryta sulfate being disintegrated by the heat, whereby it loses part of its weight. The ores are roasted to such an extent only as to remove the sulfur from the outside of the particles to render the particles more sensitive to the action of a reducing-gas, as described below. Having thus transformed the sulfids into oxids and fer-

rites by abstracting a part of the sulfur therefrom the oxids become a powerful solvent for the precious values in the ores, which then combine with the calcium-affected iron oxid. The ores are next exposed to the action of a hydrocarbon gas by being passed through a conduit or cylinder which contains such a gas. Preferably the gas is generated by dropping petroleum (oil) upon or into the heated ore; but the gas may be generated in any preferred manner. The heating of the ores as aforesaid has the effect of magnetizing the copper, nickel, and iron ores, but does not affect the zinc ores to any appreciable extent. The ores leave this conduit at a temperature of preferably about 750° centigrade and are raised by an elevator to a point where they are met by a blast of cool air, which carries them into a cooling-chamber, in which they are quickly but only partially cooled, as the copper and nickel will lose their acquired magnetism if allowed to cool too much. The bottom of the cooling-chamber is constructed to form a hopper or hoppers, through which the ores fall into one or more compound magnetic separators, the construction and operation of which will be briefly described hereinafter.

Reference is now had to the drawings, in which—

Figure 1 illustrates diagrammatically the preferred form of apparatus by which my process may be carried into effect, and Fig. 2 a detail view of the gas-conduit.

1 is a revoluble cylindrical drier, which is inclined downwardly from its receiving to its discharge end, as shown, the lower end of which communicates by a downwardly-inclined passage 2 with a roaster 3, which is shown as a revoluble cylinder; but any preferred type of roaster may be employed in lieu of the form shown. The cylindrical roaster 3 being inclined, the ores fall from its lower end, through a spout 4, into a gas conduit or cylinder 5, in which is a worm-conveyer 6, which carries the ore to one end thereof and dumps it upon an elevator 7. My preferred means for generating the hydrocarbon gas which magnetizes the gold-bearing iron ore is to drop petroleum or other hydrocarbon

oil upon the ore within said conduit 5, preferably by means of a receptacle, as 8, placed above the conduit and having a suitable opening in its bottom. (See Fig. 2.) The ore being 5 still hot from the roast vaporizes this oil which supplies the aforesaid gas.

The ores are taken up to a suitable height by the elevator 7, which dumps them into a blast-box 9, which is traversed by a powerful 10 blast of air actuated by a blower 10. The blast-box communicates with a cooling-chamber 12, in the bottom of which are preferably two hoppers 13, arranged substantially as shown. The ores are blown into this chamber, the heavier ores falling into the hopper adjacent the blast-box, while the lighter ores settle into the other hopper. In this chamber the temperature of the ores is reduced to about 250° centigrade, so that they are still 15 hot when about to be separated, which is necessary to attract the copper and nickel.

Openings covered with wire-cloth or canvas may be provided in the upper portion of this chamber for permitting the escape of the 20 heated air and gases, but preventing the escape of any of the lighter finely-divided ore.

The ores are conducted by the hoppers into any well-known form of electromagnetic separators, the forms shown in outline and briefly 25 described herein being preferred.

Beneath each hopper is placed one of my compound electromagnetic separators, each of which consists of two electromagnets mounted axially upon a vertical rotatable shaft, one 30 above the other. Each magnet is entirely inclosed within its two pole-pieces 14, which are cup-shaped and have their proximate faces or edges separated by a ring 15, of non-magnetic metal, so as to form a break in the magnetic 35 circuit. The magnets (or the pole-pieces thereof) are engaged, respectively, by two scrapers 16 and 17, which remove the adhering ores from the surfaces of the revolving pole-pieces. The lower magnet is energized more strongly 40 than the upper one to the end that the weakly-magnetized ores, as the silver-bearing ores, fall past the upper magnet and are attracted to the lower magnet, while the more strongly-magnetized ores, such as auriferous iron, 45 adhere to the upper magnet. The unmagnetized ore, such as the zinciferous, falls past both of the magnets and is received in a spout 20 or any preferred form of receptacle. The gold and silver bearing ores are separately received by 50 two spouts 18 and 19. I have made this magnet-separator the subject of a separate application for Letters Patent, the same being Serial No. 189,081, filed January 15, 1904.

By the term "crushing the ores" in the 55 claims I wish to be understood as meaning crushing, severing, or otherwise separating the ores so that they will be presented to the roaster on particles of sufficient fineness for the purpose described.

The crushing or severing of the ores may 60 be done in any desirable manner. (Not shown.)

Having thus described my invention, what I claim as new, and desire to secure by Letters Patent, is—

1. The herein-described process of treating 70 ores, consisting in, first, drying the ores; second, roasting the same; third, subjecting the heated material to the action of a hydrocarbon gas; fourth, subjecting the material to an air-blast to partially cool the same, and, fifth, passing the same through a magnetic separator. 75

2. The herein-described process of treating 80 ores consisting in, first, drying crushed ores; second, roasting and heating the same; third, subjecting the heated material to the action 85 of a hydrocarbon gas generated by the heat from the roasted ore; fourth, partially cooling the material, and, fifth, passing the same through a magnetic separator.

3. The herein-described process of treating 90 ores, consisting in, first, drying the ores; second, roasting the same; third, subjecting the material while heated to the action of a hydrocarbon gas generated by the heat from the 95 roasted ore; fourth, partially cooling the material, and, fifth, separating the magnetic components by passing the ore through magnetic fields of progressively-increased strength, whereby the strongly-magnetic ores are attracted by the lesser-energized magnetic field, and the slightly-magnetic ores by the highly-energized 100 magnetic field, substantially as described.

4. The herein-described process of treating 105 ores, consisting in, first, drying the same; second, roasting the same; third, subjecting the same to an air-blast to partially separate and cool the same, and, fourth, separating the magnetic components by passing the ore through magnetic fields of progressively-increased strength, substantially as described. 110

5. The herein-described process of treating 115 ores previously reduced to fine particles, consisting in, first, roasting the same; second, subjecting the same while heated to the action of a hydrocarbon gas; third, partially cooling the material, and, fourth, passing the same through two magnetic fields the second of which is more strongly energized than the first, substantially as described. 120

6. The herein-described process which consists in mixing with crushed ore, a portion of lime, then roasting the mixture, next subjecting the heated material to hydrocarbon gas, subsequently cooling the same partially only, and finally passing the same through a magnetic separator. 125

In testimony whereof I have hereunto signed my name in the presence of two subscribing witnesses.

ERIC HEDBURG.

Witnesses:

SAMUEL HANSON,  
ERIC F. OBORG.